

## UNITED STATES PATENT OFFICE

2,610,927

TREATMENT OF FIBROUS MATERIALS WITH  
POLYAMIDESRobinson Percy Foulds, Manchester, England,  
assignor to Tootal Broadhurst Lee Company  
Limited, Manchester, EnglandNo Drawing. Application July 29, 1947, Serial No.  
764,575. In Great Britain March 8, 1943Section 1, Public Law 690, August 8, 1946  
Patent expires March 8, 1963

5 Claims. (Cl. 117—143)

1

This invention relates to the treatment of fibrous materials especially textile fabrics with synthetic linear polyamides and is a continuation-in-part of my application Serial No. 524,105, filed February 26, 1944, and now abandoned.

Synthetic linear polyamides are known in commerce as "nylon" and are organic condensation products which contain a multiplicity of structural units linked in series by amide or thioamide groupings, produced by a process of manufacture in which non-fibre-forming organic substances of lower molecular weight are converted into products of such high molecular weight as to be capable of being formed into filaments which upon cold drawing acquire a true fibre structure recognisable by X-ray examination. When used in reference to textile art, the term "nylon" is not customarily applied to synthetic polyamides which are water-soluble. The present invention is concerned with water-insoluble, high molecular weight or fibre-forming polyamides soluble in strong acid such as are described in United States patent specification No. 2,071,250, Wallace H. Carothers, patented February 16, 1937; United States patent specification No. 2,071,253, Wallace H. Carothers, patented February 16, 1937 and United States patent specification No. 2,130,948, Wallace H. Carothers, patented September 20, 1938.

It will be apparent, therefore, that many of these synthetic linear polyamides are made from alkylene diamines and higher aliphatic dicarboxylic acids. Examples of these are polyalkylenediamine adipates and polyalkylenediamine sebacates.

Treatment of textile fabrics with solutions of water-insoluble linear polyamides in organic solvents and subsequent removal of the solvent by evaporation gives a product in which the polyamide remains behind as a film and if the quantity of polyamide is substantial, the fabric, although flexible, loses the characteristic feel and handle of a textile material. The principal object of the present invention is to deposit a water-insoluble synthetic linear polyamide on a textile fabric so that the typically textile characteristics are not lost. Another object is to produce a dull or matt finish on fibrous materials especially textile fabrics.

These objects are secured in the present invention by precipitating a water-insoluble synthetic linear polyamide on the fibrous material, especially a textile fabric, in the form of finely divided, adherent particles. Water-insoluble synthetic linear polyamides will dissolve in com-

paratively strong acid and may be precipitated therefrom by the action of an aqueous medium and this fact is utilised in the present invention to precipitate the polyamide on cellulosic or non-cellulosic fibrous materials. When so precipitated on the fibrous material, the polyamide adheres firmly to the fibres producing a white, opaque effect which is fast to laundering and does not render the fibrous material hard or harsh.

Despite the fact that synthetic linear polyamides, as is known, are hydrolysed by strong acids, I have found that the hydrolysis is so slow that it is possible to apply solutions of them in strong acids to fibrous materials and then to precipitate the polyamides on to the materials by aqueous media without any material hydrolysis taking place.

The material on which the water-insoluble linear polyamide has been precipitated can be passed with or without tension over heated rollers to fuse the polyamide. This is particularly applicable to synthetic linear polyamides of low melting point. It will be apparent from the aforementioned patent specifications that there is a wide range of water-insoluble synthetic linear polyamides of various melting points. Any of these either singly or mixed, soluble in strong acid, may be used in carrying out the present invention.

Among the fibrous materials which may be treated are cotton, linen, wool, natural silk, viscose yarn, cellulose acetate or mixtures of any of these with one another or with synthetic linear polyamide fibres but the reagent should be chosen so as not to damage the material treated. The fibrous material may be in the form of fabrics, woven or knitted, or in any other form, e. g. as yarn, fibre or sheet. Continuous sheet material such as paper or wood may also be treated with water-insoluble synthetic linear polyamides by this method.

Fabric which is treated in accordance with the present invention may be rendered crease-resistant by means of resinous condensation products and, if required, after-treated with swelling agents, or the treated fabric may be subjected to other finishing processes. Wool treated with water-insoluble synthetic linear polyamides in accordance with the present invention resists shrinking and felting after milling.

Among the strong acids which may be used are sulphuric, hydrochloric, nitric, phosphoric and formic acids but any other strong acids known to

dissolve water-insoluble synthetic linear polyamides may be used. Mineral acids, especially sulphuric acid are very convenient solvents to use. Formaldehyde may be added to a sulphuric solution if desired, especially when such solution is used for treating cotton fabrics. The concentration of the acid used must be sufficient to enable the polyamide to dissolve. The more concentrated is the acid, the more readily will the polyamide be dissolved but on the other hand the more concentrated acids hydrolyse polyamides more readily and this must be taken into consideration in the treatment of textile materials with such solutions. Moreover, the concentration of acid which can be used obviously depends upon the strength of the acid. In the case of formic acid, for example, this may be used anhydrous whereas the form of sulphuric acid commercially known as "concentrated sulphuric acid" cannot safely be used.

A convenient way of treating a textile fabric is to pass it through a solution of the polyamide in sulphuric acid, squeeze it and then run it into water, whereupon the polyamide is deposited on the fabric as a white pigment. The squeezing will generally be such as to leave 100% by weight of solution calculated on the dryweight of the fabric on the textile. Other pigments which will dissolve in the acid and will be precipitated therefrom by the addition of water (or substances soluble in the acid from which pigments are formed and precipitated by water) may be added to the solution so that co-precipitation takes place.

In order to obtain pattern effects on fabrics, a resist may be printed on the fabric before impregnation with the acid solution. An example of such resists which are preferably insoluble in strong acid, is cellulose nitrate. Other resists insoluble in strong acid are well known.

Fabrics which have been treated in accordance with the present invention may be given other known treatments such as parchmentising, for example with sulphuric acid or zinc chloride, or other known parchmentising agents, or may be waterproofed, for example with one of the known pyridinium compounds.

The invention will be more clearly understood from the following examples which illustrate various ways of practising the invention but it will be understood that the invention is not limited to these examples.

#### Example 1

2 parts by weight of polyhexamethylenediamine adipamide having a melting point of 278° C. are dissolved in 27 parts by weight of 70° Tw. sulphuric acid. A cotton or viscose fabric is run through this solution and nipped off, after which it is washed off in water and neutralised.

In the above example we may use 2 parts by weight of the polymer in 25 parts of 78° Tw. nitric acid or 10 parts by weight of the polymer in 100 parts of formic acid, instead of the sulphuric acid, with similar result.

#### Example 2

A fine cambric is run through a solution of 1 part by weight of polyethylenediamine sebacate of melting point 254° C. the manufacture of which is described in United States patent specification No. 2,130,948 in 25 parts by weight of commercial hydrochloric acid containing 3% by weight of antimony trichloride, passed through

a nip to leave 100% of solution on the fabric and then washed off in water and neutralised.

#### Example 3

2 parts by weight of polytetramethylenediamine adipamide of melting point 278° C. the manufacture of which is described in British patent specification No. 474,999, are dissolved in 27 parts by weight of 70° Tw. sulphuric acid. A cotton or viscose fabric is run through this solution and nipped off, after which it is washed off in water and neutralised. The so-treated fabric is then run through 140° Tw. sulphuric acid for 5 seconds after which it is washed off again in water and neutralised. This treatment gives a stiff parchmentised effect.

#### Example 4

2 parts by weight of an interpolyamide prepared by heating equimolecular proportions of hexamethylenediamine adipamide and decamethylene diammonium sebacate having a softening point of 112° C., the manufacture of which is described in British patent specification No. 559,514, are dissolved in 27 parts by weight of 70° Tw. sulphuric acid. A cotton or viscose fabric is run through this solution and nipped off, after which it is washed off in water and neutralised. The fabric is then run over a hot roller, with or without stretching, at a temperature high enough to melt the polyamide.

In the above example we may use commercial hydrochloric acid or nitric acid, instead of the sulphuric acid, with similar result.

#### Example 5

Paper is impregnated with a solution, in 25 parts by weight of 70° Tw. sulphuric acid, of 1 part by weight of a polymer prepared by heating hexamethylene diammonium adipate and aminostearic acid and having a melting point of 130° C. and an intrinsic viscosity of 0.98, the manufacture of which is described in British patent specification No. 559,514. The paper is then immersed in water to precipitate the polyamide thereon. Sheets of paper thus treated can be banded together by heating an assembly of them to a sufficient temperature to bond the polyamide.

#### Example 6

1 to 2 parts by weight of the polyamide prepared from pentamethylenediamine and brassic acid having a melting point of 176° C., the manufacture of which is described in United States patent specification No. 2,130,948, are dissolved or dispersed in 25 parts by weight of sulphuric acid of 70° Tw. To the solution is added loose fibre of any description after which the polyamide is precipitated with water, washed and neutralised. The mass of polyamide covered fibres is then heated above the melting point of the polyamide and pressed so that a composite mass of polyamide and fibres is obtained. Alternatively, the mass can be rolled into any required thickness and then heated to melt the polyamide either all over or in selected portions to form a pattern. Alternatively the fibres after washing and neutralising can be made into paper in the usual manner and then heated to melt the polyamide.

The details given in the foregoing examples may be altered without departing from the invention which is of the scope of the appended claims. For example, instead of using water as the precipitant for the polyamide we may use any aqueous liquor in which the polyamide is sub-

stantially insoluble and with which the solution of polyamide is miscible and which does not have any detrimental effect upon the fibrous material treated such as dilute aqueous alkali, e. g. caustic soda or aqueous solutions containing inert salts such as sodium chloride or sodium sulphate.

I declare that what I claim is:

1. Process of treating fibrous material which consists in applying to it a solution of a polyalkylenediamine adipamide in sulphuric acid, removing excess solution and then passing the material into water and thereby precipitating in situ the said polyalkylenediamine adipamide in fine particular form, and neutralising the fibrous material.

2. The process of treating fibrous material which comprises applying to it a solution of two parts by weight of polyhexamethylene-diamine adipamide in 27 parts of 70° Tw. sulphuric acid; wringing out excess solution; washing the material in water and thereby precipitating in situ the said polyhexamethylene-diamine adipamide in fine particular form, and neutralising free acid.

3. The process of treating fibrous material which comprises applying to it a solution of two parts by weight of polytetraethylene-diamine adipamide in 27 parts of 70° Tw. sulphuric acid; wringing out excess solution; washing the material in water and thereby precipitating in situ the said polytetraethylene-diamine adipamide in

fine particular form; and thereafter treating the material with a roller hot enough to melt the polyamide present thereon.

4. The process of treating fibrous material which comprises applying to it a solution containing from one to two parts by weight of water-insoluble synthetic linear polyamide derived by condensation of a polyamine with a dibasic acid dissolved in from 25 to 27 parts by weight of 70° Tw. sulphuric acid; wringing out excess solution; washing the material in water, and neutralising free acid.

5. Cotton fabric made according to the process of claim 2; and characterised in having an adherent opaque deposit in fine particular form of the polyalkylenediamine adipamide precipitated in situ.

ROBINSON PERCY FOULDS.

#### REFERENCES CITED

The following references are of record in the file of this patent:

#### UNITED STATES PATENTS

| Number       | Name      | Date          |
|--------------|-----------|---------------|
| 1,640,596    | Chatham   | Aug. 30, 1927 |
| 2,188,332    | Carothers | Jan. 30, 1940 |
| 2,302,332    | Leekley   | Nov. 17, 1942 |
| 2,342,387    | Catlin    | Feb. 22, 1944 |
| 30 2,359,878 | Schupp    | Oct. 10, 1944 |